

# United States Patent [19]

Hanlon

[11] Patent Number: 4,482,357

[45] Date of Patent: Nov. 13, 1984

[54] FUEL COMPOSITIONS

[75] Inventor: J. Vincent Hanlon, Baton Rouge, La.

[73] Assignee: Ethyl Corporation, Richmond, Va.

[21] Appl. No.: 567,090

[22] Filed: Dec. 30, 1983

[51] Int. Cl.<sup>3</sup> ..... C10L 1/22

[52] U.S. Cl. ..... 44/63; 44/71

[58] Field of Search ..... 44/57, 71, 72, 63

[56] References Cited

U.S. PATENT DOCUMENTS

2,945,749 7/1960 Andress, Jr. ..... 44/72  
3,490,882 1/1970 Dunworth ..... 44/72  
4,240,803 12/1980 Andress, Jr. ..... 44/71

Primary Examiner—Mrs. Y. Harris-Smith

Attorney, Agent, or Firm—Donald L. Johnson; John F. Sieberth; Willard G. Montgomery

[57] ABSTRACT

Coking in and around the injector nozzles of indirect injection compression ignition engines is reduced by means of distillate fuel with which has been blended suitable concentrations of:

- (a) hydrocarbyl-substituted succinimide,
- (b) hydrocarbyl amine having from 3 to 60 carbons and from 1 to 10 nitrogens, and
- (c) N,N'-disalicylidene-1,2-diaminopropane.

Also described are additive mixtures of (a), (b) and (c) for use in distillate fuels in amounts sufficient to reduce the coking tendencies of such fuels when used in the operation of indirect injection compression ignition engines.

28 Claims, 1 Drawing Figure



U.S. Patent

Nov. 13, 1984

4,482,357



## FUEL COMPOSITIONS

## FIELD

Compression ignition fuel compositions and additive mixtures of hydrocarbyl-substituted succinimide, hydrocarbyl amine having from 3 to 60 carbons and from 1 to 10 nitrogens and N,N'-disalicylidene-1,2-diaminopropane, in amounts sufficient to resist the coking tendencies of compression ignition fuel compositions when used in the operation of indirect injection diesel engines.

## BACKGROUND

Throttling diesel nozzles have recently come into widespread use in indirect injection automotive and light-duty diesel truck engines, i.e., compression ignition engines in which the fuel is injected into and ignited in a prechamber or swirl chamber. In this way, the flame front proceeds from the prechamber into the larger compression chamber where the combustion is completed. Engines designed in this manner allow for quieter and smoother operation. The FIGURE of the Drawing illustrates the geometry of the typical throttling diesel nozzle (often referred to as the "pintle nozzle").

Unfortunately, the advent of such engines has given rise to a new problem, that of excessive coking on the critical surfaces of the injectors that inject fuel into the prechamber or swirl chamber of the engine. In particular and with reference to the FIGURE, the carbon tends to fill in all of the available corners and surfaces of the obturator 10 and the form 12 until a smooth profile is achieved. The carbon also tends to block the drilled orifice 14 in the injector body 16 and fill up to the seat 18. In severe cases, carbon builds up on the form 12 and the obturator 10 to such an extent that it interferes with the spray pattern of the fuel issuing from around the perimeter of orifice 14. Such carbon build up or coking often results in such undesirable consequences as delayed fuel injection, increased rate of fuel injection, increased rate of combustion chamber pressure rise, and increased engine noise, and can also result in an excessive increase in emission from the engine of unburned hydrocarbons.

While low fuel cetane number is believed to be a major contributing factor to the coking problem, it is not the only relevant factor. Thermal and oxidative stability (lacquering tendencies), fuel aromaticity, and such fuel characteristics as viscosity, surface tension and relative density have also been indicated to play a role in the coking problem.

An important contribution to the art would be a fuel composition which has enhanced resistance to coking tendencies when employed in the operation of indirect injection diesel engines.

## THE INVENTION

In accordance with one of its embodiments, this invention provides distillate fuel for indirect injection compression ignition engines containing at least the combination of (a) hydrocarbyl-substituted succinimide, (b) hydrocarbyl amine having from 3 to 60 carbons and from 1 to 10 nitrogens and (c) N,N'-disalicylidene-1,2-diaminopropane, said combination being present in an amount sufficient to minimize coking, especially throttling nozzle coking, in the prechambers or

swirl chambers of indirect injection compression ignition engines operated on such fuel.

Another embodiment of the present invention is a distillate fuel additive fluid composition comprising (a) hydrocarbyl-substituted succinimide, (b) hydrocarbyl amine having from 3 to 60 carbons and from 1 to 10 nitrogens and (c) N,N'-disalicylidene-1,2-diaminopropane, in an amount sufficient to minimize the coking characteristics of such fuel, especially throttling nozzle coking, in the prechambers or swirl chambers of indirect compression ignition engines operated on such fuel.

Since the invention also embodies the operation of an indirect injection compression ignition engine in a manner which results in reduced coking, a still further embodiment of the present invention is a method of inhibiting coking, especially throttling nozzle coking, in the prechambers or swirl chambers of an indirect injection compression ignition engine, which comprises supplying said engine with a distillate fuel containing at least the combination of (a) hydrocarbyl-substituted succinimide, (b) hydrocarbyl amine having from 3 to 60 carbons and from 1 to 10 nitrogens and (c) N,N'-disalicylidene-1,2-diaminopropane, said combination being present in an amount sufficient to minimize such coking in an engine operated on such fuel.

A feature of this invention is that the combination of additives utilized in its practice is capable of suppressing coking tendencies of fuels used to operate indirect injection compression ignition engines. Such behavior was exhibited in a series of standard engine dynamometer tests conducted as described in Example I hereinafter.

The hydrocarbyl-substituted succinimides, component (a) of the fuels of this invention, are well known. They are readily made by first reacting an olefinically unsaturated hydrocarbon of the desired molecular weight with maleic anhydride to form a hydrocarbyl-substituted succinic anhydride. Reaction temperatures of about 100°-250° C. are used. With higher boiling olefinically-unsaturated hydrocarbons, good results are obtained at about 200°-250° C. This reaction can be promoted by the addition of chlorine. Typical olefins include cracked wax olefins, linear alpha olefins, branched chain alpha olefins, polymers and copolymers of lower olefins. These include polymers of ethylene, propylene, isobutylene, 1-hexene, 1-decene and the like. Useful copolymers are ethylene-propylene copolymers, ethylene-isobutylene copolymers, propylene-isobutylene copolymers, ethylene-1-decene copolymers and the like.

Hydrocarbyl substituents have also been made from olefin terpolymers. Very useful products have been made from ethylene-C<sub>3</sub>-12 alpha olefin-C<sub>5</sub>-12 non-conjugated diene terpolymers; such as ethylene-propylene-1,4-hexadiene terpolymer; ethylene-propylene-1,5-cyclooctadiene terpolymer; ethylene-propylenenorbornene terpolymers and the like.

Of the foregoing, by far the most useful hydrocarbyl substituents are derived from butene polymers, especially polymers of isobutylene.

The molecular weight of the hydrocarbyl substituent can vary over a wide range. It is desirable that the hydrocarbyl group have a molecular weight of at least 500. Although there is no critical upper limit, a preferred range is about 500-500,000 number average molecular weight. The more preferred average molecular weight is about 700-5,000 and most preferably about 900-3,000.

Hydrocarbyl-substituted succinimides and succinamides are made by reaction of the desired hydrocarbyl-substituted succinic anhydride with an amine having at least one reactive hydrogen atom bonded to an amine nitrogen atom. Examples of these are methyl amine, dimethyl amine, n-butyl amine, di-(n-dodecyl) amine, N-(aminoethyl) piperidine, piperazine, N-(3-aminopropyl) piperazine, and the like.

Preferably, the amine has at least one reactive primary amine group capable of reacting to form the preferred succinimides. Examples of such primary amines are n-octyl amine, N,N-dimethyl-1,3-propane diamine, N-(3-aminopropyl) piperazine, 1,6-hexane diamine, and the like.

Hydroxyalkyl amines can also be used to make the succinimide-succinamide components of the invention which contain some ester groups. These amines include ethanol amine, diethanol amine, 2-hydroxypropyl amine, N-hydroxyethyl ethylenediamine and the like. Such hydroxyalkyl amines can be made by reacting a lower alkylene oxide, such as ethylene oxide, propylene oxide or butylene oxide with ammonia or a primary or secondary amine such as ethylene diamine, dethylene triamine, triethylene tetramine, tetraethylenepentamine and the like.

A more preferred class of primary amines used to make the succinimide, succinamide or mixtures thereof are the polyalkylene amines. These are polyamines and mixtures of polyamines which have the general formula



wherein R is a divalent aliphatic hydrocarbon group having 2-4 carbon atoms and n is an integer from 1-10 including mixtures of such polyalkylene amines.

In a highly preferred embodiment, the polyalkylene amine is a polyethyleneamine containing about 2-6 ethyleneamine units. These are represented by the above formula in which R is the group  $-\text{CH}_2\text{CH}_2-$  and n has a value of 2-6.

The amine used to make the succinimide, succinamide or mixture thereof need not be all amine. A mono or poly-hydroxyalcohol may be included in the reaction. Such alcohols can be reacted concurrently with the amine or the two alcohol and amine may be reacted sequentially. Useful alcohols are methanol, ethanol, n-dodecanol, 2-ethyl hexanol, ethylene glycol, propylene glycol, diethylene glycol, 2-ethoxy ethanol, trimethylol propane, pentaerythritol, dipentaerythritol and the like.

Useful amine-alcohol products are described in U.S. Pat. Nos. 3,184,474; 3,576,743; 3,632,511; 3,804,763; 3,836,471; 3,936,480; 3,948,800; 3,950,341; 3,957,854; 3,957,855; 3,991,098; 4,071,548 and 4,173,540.

The reaction between the hydrocarbyl-substituted succinic anhydride and the amine can be carried out by mixing the components and heating the mixture to a temperature high enough to cause a reaction to occur but not so high as to cause decomposition of the reactants or products or the anhydride may be heated to reaction temperature and the amine added over an extended period. A useful temperature is about 100°-250° C. Best results are obtained by conducting the reaction at a temperature high enough to distill out water formed in the reaction.

A preferred succinimide-succinamide component is available as an article of commerce from the Edwin Cooper Company under the designation HITEC®E-644. This product comprises a mixture of active ingredi-

ents and solvent. Thus, when HITEC®E-644 is used as component (a) in formulating the fuels of this invention, the product as received should be used at a concentration of at least about 40 PTB (pounds per thousand barrels) to insure that the finished blend contains an adequate quantity of the foregoing succinimide-succinamide ingredient, although smaller amounts may be successfully employed.

While a variety of hydrocarbyl amines, component (b), may be used in the fuel compositions of this invention, a primary aliphatic amine, the aliphatic group of which is tertiary, e.g., an amine of the formula:



wherein R is one or a mixture of tertiary aliphatic groups containing 8 to 18 or more (preferably 12 to 16) carbon atoms is preferred. Most preferably, these tertiary aliphatic groups are tertiary alkyl groups. It is also preferred that hydrocarbyl amine component (b) include in addition to the above-described amine one or more hydrocarbyl amines differing therefrom.

U.S. Pat. No. 3,909,215, all disclosures of which is incorporated herein, gives a description of the various hydrocarbyl amines having from 3 to 60 carbons and from 1 to 10 nitrogens which may be employed in the fuels of this invention. A few additional examples of desirable amines include 2,6-di-tert-butyl- $\alpha$ -dimethylamino-p-cresol, N-cyclohexyl-N,N-dimethylamine, and N-alkyl,N,N-dimethylamines in which the alkyl group is one or a combination of alkyl groups preferably having 8 to 18 or more carbon atoms.

A particularly preferred hydrocarbyl amine is available commercially from the Rohm and Haas Company under the designation Primene 81R. The Primene 81R is believed to be a mixture of primary aliphatic amines in which the aliphatic groups are predominantly C<sub>12</sub> and C<sub>14</sub> tertiary alkyl groups.

The fuels of this invention should contain at least 1.5 to 40 PTB of component (b), the hydrocarbyl amine.

Component (c) of the fuels of this invention is a metal deactivator. Examples of these are salicylidene-o-aminophenol, disalicylidene ethylenediamine and disalicylidene propylenediamine. A particularly preferred metal deactivator is N,N'-disalicylidene-1,2-diaminopropane (80 weight percent active in 20 weight percent toluene solvent) which is available as an article of commerce from Ethyl Corporation under the designation "Ethyl" MDA.

The fuels of this invention should contain at least 0.2 to 5 PTB of component (c), the metal deactivator, preferably N,N'-disalicylidene-1,2-diaminopropane.

It is not believed that there is anything critical as regards the maximum amount of components (a), (b) and (c) used in the fuel. Thus, the maximum amount of these components will probably be governed in any given situation by matters of choice and economics.

The coking-inhibiting components (a), (b) and (c) of the invention can be added to the fuels by any means known in the art for incorporating small quantities of additives into distillate fuels. Components (a), (b) and (c) can be added separately or they can be combined and added together. It is convenient to utilize additive fluid mixtures which consist of hydrocarbyl-substituted succinimide-succinamide agents, hydrocarbyl amine and N,N'-disalicylidene-1,2-diaminopropane. These additive fluid mixtures are added to distillate fuels. In

other words, part of the present invention are coking inhibiting fluids which comprise hydrocarbyl-substituted succinimide-succinamide, hydrocarbyl amine having from 3 to 60 carbons and 1 to 10 nitrogens, and metal deactivator, preferably N,N'-disalicylidene-1,2-diaminopropane.

Use of such fluids in addition to resulting in great convenience in storage, handling, transportation, blending with fuels, and so forth, also are potent concentrates which serve the function of inhibiting or minimizing the coking characteristics of compression ignition distillate fuels used to operate indirect compression ignition engines.

In these fluid compositions, the amount of components (a), (b) and (c) can vary widely. In general, the fluid compositions contain about 10 to 97.9% by weight of the hydrocarbyl-substituted succinimide-succinamide component, about 20 to about 75% by weight of the hydrocarbyl amine and about 0.1 to 15% by weight metal deactivator. Typically, from about 0.01% by weight up to about 1.0% by weight of the combination will be sufficient to provide good coking-inhibiting properties to the distillate fuel. A preferred distillate fuel composition contains from about 0.1 to about 0.5% by weight of the combination containing from about 50% to about 97.9% by weight of the hydrocarbyl succinimide-succinamide component and from about 2.0% to about 45% by weight of the hydrocarbyl amine and from about 0.1 to about 5.0% by weight of the metal deactivator, preferably N,N'-disalicylidene-1,2-diaminopropane.

The additive fluids, as well as the distillate fuel compositions of the present invention may also contain other additives such as, corrosion inhibitors, antioxidants, metal deactivators, detergents, cold flow improvers, inert solvents or diluents, and the like.

The practice and advantages of this invention will become still further apparent from the following illustrative example.

#### EXAMPLE 1

In order to determine the effect of the fuel compositions of the present invention on the coking tendency of diesel injectors in indirect injection compression ignition engines, use was made of a commercial diesel engine operated on a coking test cycle developed by Institute Francais Petrole and as practiced by Peugeot S. A. The amount of coking together with a quantitative indication of the adverse consequences of such coking was determined by means of (i) injector air flow performance, (ii) emission of unburned hydrocarbons, (iii) engine noise, and (iv) injector deposit ratings. The engine employed in the tests was a 1982 Peugeot 2.3 liter, 4-cylinder, turbocharged XD2S diesel engine connected to a Midwest dynamometer through an engine clutch. This engine is equipped with Bosch injectors positioned within prechambers, and is deemed representative of the indirect injection compression ignition engines widely used in automobiles and light-duty trucks.

The base fuel employed in these engine tests was a commercially-available diesel fuel having a nominal cetane rating of 42. FIA analysis indicated the fuel was composed by volume of 31.5% aromatics, 3.0% olefins and 65.5% saturates. Its distillation range (ASTM D-158) was as follows:

|                | Barometer<br>Initial<br>% Evaporated | 29.46 inches of Hg<br>406° F.<br>at °F. |
|----------------|--------------------------------------|-----------------------------------------|
| 5              | 5                                    | 439                                     |
| 10             | 10                                   | 450                                     |
| 15             | 15                                   | 456                                     |
| 20             | 20                                   | 463                                     |
| 30             | 30                                   | 480                                     |
| 40             | 40                                   | 499                                     |
| 50             | 50                                   | 521                                     |
| 60             | 60                                   | 545                                     |
| 70             | 70                                   | 572                                     |
| 80             | 80                                   | 603                                     |
| 85             | 85                                   | 621                                     |
| 90             | 90                                   | 643                                     |
| 95             | 95                                   | 678                                     |
| Final Recovery |                                      | 678° F.                                 |
| Residue        |                                      | 97.5%                                   |
| Loss           |                                      | 2.5%                                    |
|                |                                      | None                                    |

Other inspection data on the base fuel were as follows:

|                                   |                          |
|-----------------------------------|--------------------------|
| Kinematic Viscosity, (ASTM D-445) | 3.50 Centistokes, 40° C. |
| Pour Point (ASTM D-97)            | -26° C.                  |
| Cloud Point (ASTM D-97)           | 33° C.                   |
| Flash Point (ASTM D-93)           | 91° C.                   |
| Steam Jet Gum                     | 2.4 mg/100 ml            |
| Aniline Point (ASTM D-611)        | 143.4° F.                |
| Total Sulfur                      | 0.41 wt. %               |
| Ramsbottom Carbon, % (ASTM D-524) | 0.1460 on 10% Residuum   |
| Gravity (ASTM D-287)              | 31.8 °API                |
| Specific Gravity @ 25° C.         | 0.86                     |
| Cetane rating                     | 41                       |

A test blend was prepared from this base fuel (Fuel A). Fuel A contained a combination of (i) 41 PTB of HITEC ®E-644, a product of Edwin Cooper, Inc., believed to be a hydrocarbyl succinimide-succinamide made by reacting two moles of a polyisobutylene succinic anhydride (PIBSA) with one mole of a polyethylene amine mixture having an average composition corresponding to tetraethylene pentamine, (ii) 14 PTB of a hydrocarbyl amine available commercially from Rohm and Haas Company under the designation Primene 81R, and (iii) 1.7 PTB of "Ethyl" Metal Deactivator, a product of Ethyl Corporation, the active ingredient of which is N,N'-disalicylidene-1,2-diaminopropane. The manufacturer gives the following typical properties for its HITEC ®E-644 product:

|                                  |                           |
|----------------------------------|---------------------------|
| Appearance                       | Dark brown viscous liquid |
| Nitrogen, wt. %                  | 2.0                       |
| Specific Gravity<br>at 60/60° F. | 0.928                     |
| Viscosity at 210° F.,<br>cs      | 340                       |

The Primene 81R is believed to be a mixture of primary aliphatic amines in which the aliphatic groups are predominantly C<sub>12</sub> and C<sub>14</sub> tertiary alkyl groups.

The manufacturer gives the following typical properties for its "Ethyl" metal Deactivator:

|                         |        |
|-------------------------|--------|
| Form                    | Liquid |
| Color                   | Amber  |
| Density, at 68° F.      |        |
| g/ml                    | 1.0672 |
| lb/gal                  | 8.91   |
| Active ingredient, wt % | 80     |

-continued

|                                 |                                     |
|---------------------------------|-------------------------------------|
| Solvent vehicle (toluene), wt % | 20                                  |
| Flash point, open cup, °F.      | 84                                  |
| Fire point, °F.                 | 100                                 |
| <u>Solubility</u>               |                                     |
| In gasoline (Typical)           | Saturated solution contains 94% MDA |
| In water, wt. %                 | 0.04                                |

Shell Rotella T, an SAE 30, SF/CD oil was used as the crankcase lubricant.

Before starting each test, new Bosch DNOSD-1510 nozzles were installed using new copper gaskets and flame rings. The fuel line was flushed with the new test fuel composition to be tested and the fuel filter bowl and fuel return reservoir were emptied to avoid additive carry-over from test-to-test.

At the start of each test, the engine was operated at 1000 rpm, light load for 15 minutes. After this warm-up, the engine was subjected to the following automatic cycle:

| Event | RPM  | Beam Load | Minutes | EGR |
|-------|------|-----------|---------|-----|
| 1     | 750  | 0         | 4       | off |
| 2     | 2750 | 12.0      | 6       | on  |
| 3     | 1500 | 6.2       | 6       | on  |
| 4     | 4000 | 16.2      | 4       | off |

The above 20-minute cycle was repeated 60 times and the test was completed by running the engine at idle for another 30 minutes. The total elapsed time was thus 20.5 hours per test.

When passing from one event to the next event in the above cycle, some time, of course, was required to enable the engine to accelerate or decelerate from one speed to the next. Thus, more specifically, the above cycle was programmed as follows:

| Segment | Seconds | rpm  | Beam Load |
|---------|---------|------|-----------|
| 1       | 2       | 750  | 0         |
| 2       | 200     | 750  | 0         |
| 3       | 3*      | 2500 | 12        |
| 4       | 7*      | 2750 | 12        |
| 5       | 350     | 2750 | 12        |
| 6       | 3*      | 2275 | 6.2       |
| 7       | 7*      | 1500 | 6.2       |
| 8       | 330     | 1500 | 6.2       |
| 9       | 3*      | 3500 | 16.2      |
| 10      | 7*      | 4000 | 16.2      |
| 11      | 230     | 4000 | 16.2      |
| 12      | 3*      | 2000 | 0         |
| 13      | 7*      | 750  | 0         |
| 14      | 30      | 750  | 0         |

\*Represents two mode periods for acceleration or deceleration to the next condition.

Hydrocarbon exhaust emissions were measured at the start of each test (after the first 20-minute cycle), at the 6-hour test interval and at the end of the test. These measurements were made at 750, 1000, and 1400 rpm idle. Noise level readings were made at a location three feet from the engine exhaust side. The measurements were made at the start and at the end of the test while operating at three idle speeds, viz., 750, 1000 and 1400 rpm.

After the test operation, the injectors were carefully removed from the engine so as not to disturb the deposits formed thereon. Measurements were made of air flow through each nozzle at different pintle lifts, and

pintle deposits were rated using the CRC deposit rating system.

The most significant test results are given in Table I, in which air flow is expressed as cc/min and hydrocarbon emissions as ppm.

TABLE I

| Fuel | Air Flow @ 0.1 mm Lift | Pintle Obtrurator Deposits (10 = clean) | Noise, DB |       | Hydrocarbon Emissions |       |
|------|------------------------|-----------------------------------------|-----------|-------|-----------------------|-------|
|      |                        |                                         | EOT*      | INCR. | EOT*                  | Incr. |
| Base | 36                     | 8.0                                     | 83.8      | 3.0   | 577                   | 406   |
| A    | 40                     | 8.5                                     | 83.2      | 3.0   | 513                   | 278   |

\*Value at end of test; the increase (Incr.) shown is in comparison to the value at start of test.

The results presented in Table I show that there were less coking deposits (higher air flow rate and fewer deposits), less engine noise and less hydrocarbon emissions with Fuel A, the fuel of the invention, as compared to the Base Fuel.

I claim:

1. Distillate fuel for indirect injection compression ignition engines containing at least the combination of (a) hydrocarbyl-substituted succinimide or succinamide, (b) hydrocarbyl amine having from 3 to 60 carbons and from 1 to 10 nitrogens and (c) N,N'-disalicylidene-1,2-diaminopropane, said combination being present in an amount sufficient to minimize coking on the nozzles of indirect injection compression ignition engines operated on such fuel.

2. The composition of claim 1 wherein said hydrocarbyl-substituted succinimide is an olefin polymer-substituted succinimide wherein said olefin polymer substituent has an average molecular weight of about 500-500,000.

3. The composition of claim 2 wherein the succinimide portion is derived from a polyalkylene amine having the formula



wherein R is a divalent aliphatic hydrocarbon group having 2-4 carbon atoms and n is an integer from 1-10 including mixtures of said polyalkylene amines.

4. The composition of claim 3 wherein said olefin polymer substituent is a polyisobutene substituent.

5. The composition of claim 4 wherein said polyisobutene substituent has an average molecular weight of about 700-5,000.

6. The composition of claim 5 wherein said polyalkylene amine is a polyethylene amine.

7. The composition of claim 6 wherein said polyethylene amine contains about 2-6 ethylene amine units.

8. The composition of claim 1 wherein said hydrocarbyl amine is comprised of an alkylene amine of the formula



wherein R is one or a mixture of tertiary alkyl groups containing 8 to 18 carbon atoms.

9. The composition of claim 8 wherein R is one or a mixture of tertiary alkyl groups containing 12 to 16 carbon atoms.

10. A process of inhibiting coking on the injector nozzles of an indirect injection compression ignition engine, which method comprises supplying said engine with a distillate fuel containing at least the combination of (a) hydrocarbyl-substituted succinimide or succinam-

ide, (b) hydrocarbyl amine having from 3 to 60 carbons and from 1 to 10 nitrogens and (c) N,N'-disalicylidene-1,2-diaminopropane, said combination being present in an amount sufficient to minimize such coking in the engine operated on such fuel.

11. The process of claim 10 wherein said hydrocarbyl-substituted succinimide is an olefin polymer-substituted succinimide wherein said olefin polymer substituent has an average molecular weight of about 500-500,000.

12. The process of claim 11 wherein the succinimide portion is derived from a polyalkylene amine of the formula



wherein R is a divalent aliphatic hydrocarbon group having 2-4 carbon atoms and n is an integer from 1-10 including mixtures of said polyalkylene amines.

13. The process of claim 12 wherein said olefin polymer substituent is polyisobutene substituent.

14. The process of claim 13 wherein said polyisobutene substituent has an average molecular weight of about 700-5,000.

15. The process of claim 14 wherein said polyalkylene amine is a polyethylene amine.

16. The process of claim 15 wherein said polyethylene amine contains about 2-6 ethylene amine units.

17. The process of claim 10 wherein said hydrocarbyl amine is comprised of alkyl amine of the formula



wherein R is one or a mixture of tertiary alkyl groups containing 8 to 18 or more carbon atoms.

18. The process of claim 17 wherein R is one or a mixture of tertiary alkyl groups containing 12 to 16 carbon atoms.

19. An additive fluid concentrate for use in distillate fuels containing at least the combination of (a) a hydrocarbyl-substituted succinimide or succinamide, (b) hydrocarbyl amine having from 3 to 60 carbons and from

1 to 10 nitrogens and (c) N,N'-disalicylidene-1,2-diaminopropane.

20. A concentrate of claim 19 wherein said hydrocarbyl-substituted succinimide is an olefin polymer-substituted succinimide wherein said olefin polymer substituent has an average molecular weight of about 500-500,000.

21. A concentrate of claim 20 wherein the succinimide portion is derived from polyalkylene amine having the formula



wherein R is a divalent hydrocarbon aliphatic group having 2-4 carbon atoms and n is an integer from 1-10 including mixtures of said polyalkylene amines.

22. A concentrate of claim 21 wherein said olefin polymer substituent is a polyisobutene substituent.

23. A concentrate of claim 22 wherein said polyisobutene substituent has an average molecular weight of about 700-5,000.

24. A concentrate of claim 23 wherein said polyalkylene amine is a polyethylene amine.

25. A concentrate of claim 24 wherein said polyethylene amine contains about 2-6 ethylene amine units.

26. A concentrate of claim 19 wherein said hydrocarbyl amine is comprised of an alkylene amine of the formula



wherein R is one or a mixture of tertiary alkyl groups containing 8 to 18 carbon atoms.

27. A concentrate of claim 26 wherein R is one or a mixture of tertiary alkyl groups containing 12 to 16 carbon atoms.

28. A concentrate of claim 19 comprising from about 10 to 97.9% by weight of said hydrocarbyl-substituted succinimide or succinamide, 2.0 to 75% by weight of said hydrocarbyl amine and 0.1 to 15% by weight of said N,N'-disalicylidene-1,2-diaminopropane.

\* \* \* \* \*